

## UNITED STATES PATENT OFFICE

2,608,492

## INSULATION BOARD

Margaret E. Mueller, New York, N. Y.

No Drawing. Application December 19, 1944,  
Serial No. 568,941

5 Claims. (Cl. 106—163)

1

The invention relates to improvements in fibrous building material and processes for making the same. More particularly, it relates to the production of an inexpensive improved fibrous insulation and building board having great strength and excellent insulating qualities.

As a basic material for the formation of the boards of the invention, the shives forming the waste material after decorticating flax and hemp stalks and the like are of particular advantage. Ordinarily, before the decorticating of flax and hemp and other bast fiber plants, the stalks are exposed to the weather or soaked in water in order to facilitate the removal of the bast fibers for spinning and other purposes. This process is known as retting and in the course of the process there is a considerable loss of plant juices containing many of the constituents both of the bark and the shives. Among these constituents so lost in great part are pentosan and furfural, and also natural resins, all of which are of particular importance as natural binding material in the formation of the boards.

In the manufacture of the board of the present invention, it is a particular object to utilize these natural binders and it is, therefore, desirable that the shives or woody portion of the plant used for the purpose should be derived from unretted stalks of flax and hemp and other bast fiber plants and grasses. At the present time, processes are known for decorticating flax and hemp without retting and the shives resulting from these processes contain practically all the furfural and pentosan and also cellulose and lignin as well as the resinous materials of the natural stalks. Flax and hemp shives, for instance, are very similar in chemical composition. Analysis shows the following percentages:

|                     | Flax  | Hemp  |
|---------------------|-------|-------|
| Resins.....         | 3.58  | 2.85  |
| Furfural.....       | 14.07 | 14.18 |
| Pentosan.....       | 24.01 | 24.16 |
| Pure Cellulose..... | 37.05 | 40.57 |

and the rest is largely lignin and inert materials. Largely due to the higher percentages of these constituents in hemp, the hemp shives make a stronger board than flax shives. It will be understood that in the case of all these fiber plants, the invention contemplates the formation of the boards without the addition of any binders or fillers other than those contained in the material itself.

While ordinarily the shives do not need to be

2

broken up or otherwise processed beyond what takes place in the decorticating machinery, where it is desired to produce a finer grained board, the shives may be cut, shredded or ground.

The material, with an adequate amount of water to float the same, is put into beaters and reduced to a pulp of somewhat coarser nature than would be used for making the better grades of paper. It is reduced in the beaters to about 5 the condition of half stock at a temperature of about 125° to 150° F.

The pulp may be then spread to a predetermined thickness on a screen and is then pressed to squeeze out a large proportion of the water contained therein, and the body so formed is then subjected to pressure of about 100-200 lbs. per square inch while it is heated to a temperature of about 150° to 200° F. and the board is pressed to its final thickness, precautions being taken to 10 prevent lateral expansion thereof. It is then placed in a drier and dried at a temperature of about 200° to 250° F. During this process the natural binding materials in the shives are released and permeate the entire board and the 15 pressure and heating are maintained until the board is practically dry, the heat and pressure being maintained until all danger of warping is past. A smooth, strong board results that can be used as a wall board or interior woodwork or as heat insulation in a building or in refrigerators, 20 as desired.

Having thus described my invention, what I claim is:

1. A composition of matter consisting of woody material derived from the shives of unretted bast fiber plants containing substantially all the natural content of pentosan and furfural-yielding material and pressed under heating into the form of an insulating and building board.
2. An insulation and building board composed of untreated hemp shives containing substantially all the pentosan and furfural-yielding material of such shives as a bonding material and formed under heat and pressure.
3. An insulation and building board composed of hemp shives containing substantially all of the natural pentosan and furfural-yielding material of said shives and formed under conditions of moisture, heat and pressure.
4. An insulation and building board consisting of a strong, stiff body of woody material composed of the shives of unretted flax containing substantially all the pentosan and furfural-yielding material of said shives as a bonding material.

5. An insulation and building board consisting of the shives of unretted flax containing substantially all the pentosan and furfural-yielding material of said shives as a binder for the fiber of said unretted flax.

MARGARET E. MUELLER.

REFERENCES CITED

The following references are of record in the file of this patent:

UNITED STATES PATENTS

| Number    | Name   | Date          |
|-----------|--------|---------------|
| 908,681   | Lappen | Jan. 5, 1909  |
| 1,108,155 | Ellis  | Aug. 25, 1914 |
| 1,503,211 | Shaw   | July 29, 1924 |

| Number      |
|-------------|
| 1,623,184   |
| 1,718,011   |
| 1,803,737   |
| 5 1,941,817 |
| 2,317,394   |

| Name           | Date          |
|----------------|---------------|
| Hinde          | Apr. 5, 1927  |
| Vogt           | June 18, 1929 |
| Sweeney        | May 5, 1931   |
| Sweeney et al. | Jan. 2, 1934  |
| Mason et al.   | Apr. 27, 1943 |

FOREIGN PATENTS

| Country       | Date          |
|---------------|---------------|
| Great Britain | of 1855       |
| Great Britain | of 1857       |
| Great Britain | Aug. 6, 1931  |
| Australia     | Oct. 19, 1939 |
| France        | Feb. 12, 1917 |
| France        | Feb. 3, 1928  |